

Nov. 14, 1944.

E. H. BALZ ET AL

2,362,528

## PREPARATION OF FINE CELLULOSE FLOUR

Filed June 3, 1942



Emil H. Balz  
Andrew W. Kassay INVENTORS  
William D. Williams

BY  
Marshall & Marshall  
ATTORNEYS

## UNITED STATES PATENT OFFICE

2,362,528

## PREPARATION OF FINE CELLULOSE FLOUR

Emil H. Balk, Andrew W. Kassay, and William D. Williams, Toledo, Ohio, assignors, by mesne assignments to Libbey-Owens-Ford Glass Company, a corporation of Ohio

Application June 3, 1942, Serial No. 445,656

2 Claims. (Cl. 83—94)

The invention relates to the preparation of fine cellulose flour that is useful as a filler for synthetic resin compositions, such as molding compounds and adhesives, and other products, such as insecticides, for which fine cellulose flour is now used.

Wood and other forms of cellulose are difficult to reduce to a fine powder because of the fibrous nature of cellulose. Cellulose is a tough and flexible material, and the individual cellulose fibers are believed to have a higher tensile strength than steel. For many applications extremely fine cellulose flour is desirable, and such cellulose flour is difficult to produce by grinding because of the toughness of the cellulose fibers.

Cellulose can be reduced to a fine flour by prolonged grinding in a tumbling impact mill in which the cellulose is ground by the impact of tumbling members, such as a ball mill or a tube mill. A ball mill consists essentially of a rotary cylinder containing steel or porcelain balls which tumble as the cylinder rotates and exert a grinding action upon material contained in the cylinder. In a continuous process a grinding operation of this character is ordinarily performed by a tube mill. Tumbling members in the form of tubes or rods may be employed in place of balls in such a mill. A continuous mill of this type is an elongated cylinder rotating on its longitudinal axis, which is inclined slightly so that when material is fed at the higher end, the ground product will flow at the lower end.

Such a tumbling impact mill must be of relatively large size in order to provide a reasonable out-put because the material passes through the mill quite slowly. Thus a tumbling impact mill is a very expensive piece of production equipment. However, a tumbling impact mill is the only type of mill in which cellulose can be ground to a fine flour.

A common form of commercial mill, known as an attrition mill, is ordinarily employed for the operation of reducing a fine saw-dust to the form of coarse wood flour. The finest wood flour that can be produced by means of an attrition mill is so coarse that less than 5 per cent of it will pass through a 100 mesh screen. The fine wood flour that is desired for most applications of the type mentioned above is wood flour so fine that substantially all of it will pass through a 270 mesh screen.

The principal object of the invention is to provide a method of producing cellulose flour by which a tumbling impact mill of relatively small size can be used to provide a relatively large out-

put of cellulose flour. More specific objects and advantages are apparent from the description in which reference is had to the accompanying drawing.

Figure I of the drawing illustrates a preferred form of apparatus for carrying out the invention.

Figure II is a vertical section taken on the line II—II of Figure I.

This specific drawing and the specific description that follows merely disclose and illustrate the invention, and are not intended to impose limitations upon the claims.

After cellulose has been ground in a ball mill or other tumbling impact mill for several hours, only a small proportion of particles finer than the meshes in a 270 mesh screen can be recovered, and it is necessary to prolong the grinding in the tumbling impact mill for an unreasonable length of time in order to reduce the greater proportion of the cellulose to a flour of such fineness.

In accordance with the invention, it has been discovered that fine cellulose particles cannot be satisfactorily separated from coarser cellulose particles by screening. Cellulose particles which are fine enough to pass through the meshes of a screen, because of their fibrous nature, interlock together and bridge over the meshes of the screen. Dry screening thus provides an unsatisfactory separation of the desired fine particles. Effective separation by screening can be accomplished if the ground cellulose is made up in a slurry with water and screened wet. Such satisfactory screening is not an economical operation, however, because of the expense of making up the slurry and subsequently drying the product.

In accordance with the invention, therefore, the desired fine particles are removed from the ground mass in each step by air separation. The invention is based upon the discovery that even air separation does not provide satisfactory removal of the fine particles. It has been discovered that because of static charges on the fine particles or because of enmeshing fibrous tentacles on the particles, there is a tendency for groups of fine particles to cling together in clumps. Such clumps do not go off with the fine particles when air separation is carried out, but are removed with the coarse particles or tailings. It has been discovered that if the tailings from such an air separation are subjected to a simple grinding operation, the clumps of fine particles become separated so that a large yield of additional fines can be obtained by a further air separation. Thus when a yield of 20 per cent fines is obtained by air separation of cellulose that has

been ground in a ball mill, an additional yield of an equal or greater amount of fines can be obtained by passing the tailings from such air separation through a simple grinder of the usual rotor impact type and again air separating.

The invention is thus carried out by grinding cellulose in a tumbling impact mill, air-separating the fines from the resulting product, re-grinding the tailings from the air separation, and air-separating the fines from the material so reground. Preferably the tailings from the first air separation are re-ground in an imp mill, which is a simple type of rotor impact mill, and the tailings from the second air separation are returned to the tumbling impact mill.

The principal application of the invention is in the production of fine wood flour. In the production of wood flour by the present method, fine saw-dust, obtained by passing chips, shavings and coarse saw-dust through a rotary cutter, is ground in an attrition mill to produce coarse wood flour which is in turn fed to the tumbling impact mill used in carrying out the present invention. The present method can be used for comminuting any form of cellulose, such as walnut shell, flax shives, a bleached sulfite pulp, such as alpha cellulose, or any other cellulosic material.

When the method is carried out by means of the apparatus illustrated in the drawing, wood waste, usually in the form of a mixture of chips, shavings and coarse saw-dust, is passed through a rotary cutter 1 which converts it to fine saw-dust. The fine saw-dust is suitable for processing in an attrition mill 2 to which it is conducted by a chute 3. The attrition mill reduces the fine saw-dust to a coarse wood flour. The attrition mill is used to effect a preliminary grinding of the material in order to make possible a more rapid out-put from the tube mill 4 to which the coarse wood flour is fed from the attrition mill through an inclined chute 5. Although the attrition mill is capable of carrying out only a preliminary and relatively coarse grinding of the material, the out-put of a small attrition mill in pounds per hour is greater than the out-put of a large tube mill costing 20 to 30 times as much as the attrition mill.

The tube mill 4 should be provided with a jacket of the usual type, for cooling water.

The ground product is discharged from the tube mill 4 into a storage hopper 6 provided with a gate 7. From time to time the gate 7 is opened slightly to cause the contents of the hopper 6 to be emptied slowly into a chute 8 from which the

product is conveyed pneumatically by a blower 9 through a conduit 10 to an air separator 11. The surplus air from the air separator 11 returns through ducts 12 and 13 to the blower 9. A bag 14 is used to collect the fines, which are the finished product. After each emptying of the storage hopper 6, the gate 7 is closed, a gate 15 in a tailings hopper 16 is opened and a diverting vane 17 is turned to the left in order to cause the tailings from the hopper 16 to be fed to a small imp mill 18, having an impact rotor 18a. By means of a blower 19 the product from the imp mill 18 is conveyed pneumatically through a vertical conduit 20 to the air separator 11, and the surplus air from the air separator is returned to the blower 19 through the return air ducts 12 and 21. A gate 22 in the discharge chute 23 for the fines is provided in order to permit the discharge of the fines to be shut off momentarily while an empty bag is substituted for a full bag. The re-grinding of the tailings in the imp mill 18 and the air separation of the resulting product are continued, the tailings from the second air separation being returned to the imp mill, until the discharge of fines from the air separator has substantially ceased. Then the diverting vane 17 is turned to the right and the grinding of the tailings in the imp mill and air separation of the resulting product are continued until all of the tailings have been fed back to the tube mill 4. The gate 15 of the tailings hopper 16 is then closed, and the system is ready for another emptying of the storage hopper 6.

Various embodiments may be devised to meet 35 various requirements.

Having described the invention, we claim:

1. A method of producing cellulose flour that comprises grinding cellulose in a tumbling impact mill, air-separating the fines from the resulting product, regrinding the tailings from the air separation in a rotor impact mill, and air-separating the fines from the material so reground.

2. A method of producing cellulose flour that comprises grinding cellulose in a tumbling impact mill, air-separating the fines from the resulting product, regrinding the tailings from the air separation in a rotor impact mill, air-separating the fines from the material so reground, and returning to said tumbling impact mill the tailings from the second air separation.

EMIL H. BALZ.  
ANDREW W. KASSAY.  
WILLIAM D. WILLIAMS.